

Dec. 6, 1932.

F. G. CRANE

1,889,851

METHOD OF MAKING AND TREATING PAPER

Filed Jan. 10, 1931



INVENTOR  
Frank G. Crane  
BY  
Chappell & Land  
ATTORNEYS.

## UNITED STATES PATENT OFFICE

FRANK G. CRANE, OF MONTAGUE, MICHIGAN

## METHOD OF MAKING AND TREATING PAPER

Application filed January 10, 1931. Serial No. 507,802.

The main objects of this invention are:

First, to provide an improved method of making paper which results in a superior product and at the same time reduces the cost 5 of production.

Second, to provide a method of making or treating paper which results in a product having the qualities of coated paper, which is very flexible and may be repeatedly folded 10 without cracking as ordinarily results from heavy coated papers.

Third, to provide a method of producing paper having these advantages in which light weight papers may be produced or 15 treated to render them entirely opaque.

Fourth, to provide a method of producing paper having the advantages of coated paper produced by the usual methods which eliminates the coating apparatus, drying 20 rooms, and materials commonly employed in the industry.

Objects pertaining to details and economies 25 of my invention will definitely appear from the description to follow. The invention is defined in the claims.

The manner of carrying out my invention is illustrated in the accompanying drawing, in which Figs. 1 and 2 are complementary 30 diagrammatic conventionalized illustrations of an apparatus which may be employed in the practice of my method or process.

In this drawing 1 represents a paper making machine of the Fourdrinier type, 2 a 35 group of drying rolls and 3 a second group of drying rolls, both of which are operatively associated with the paper making machine. 4 represents a calendering machine which is operatively associated with the second set of 40 drying rolls.

Between the sets of drying rolls 2 and 3 I interpose an apparatus for performing certain steps of my process. This apparatus comprises a tank 5 disposed at the rear of the 45 drying rolls 2 having guide rollers 6 and 7 arranged therein so that the web of paper indicated at 8 is passed from the drying cylinders 2 into the solution or liquid contained within the tank 5. A set of gaging rollers 9 is arranged to act on the web as it passes from the

tank 5, one of these rollers being provided with screw adjusting means.

From the tank 5 the web passes into a second tank 10 which has guide rollers 11 and 12 arranged therein to guide the web through 55 the solution within the tank, and is preferably provided with a set of squeeze or gaging rollers 13.

It is desired to state, however, that certain 60 steps of my improved method may be practiced with paper that has been previously formed and completely dried; that is, the paper web is formed as a separate step instead of part of the continuous operation as is possible with the apparatus illustrated. 65

My improved method comprises forming 70 the paper without filler, sizes or precipitant such as are the common practice where the sizing and filler are added to the stock prior to forming the web. The web is partially dried as by means of drying cylinders indicated at 2 on the drawing, and is then passed into a bath or solution comprising silicate of 75 soda, starch or other suitable binder, glycerin and soap. The following proportions will be found very satisfactory: silicate of 80 soda, approximately 50%; starch or other binder, approximately 25%; glycerin, approximately 15%; soap, approximately 10%, preferably in the form of white or uncolored 85 soap chips.

The guide rollers 6 and 7 are provided to insure the submerging of the web in the solution and the web is entirely impregnated during its passage through the solution. As it 85 passes from the tank 5 it is acted upon by the gaging or squeezing rollers 9 which remove the excess and should be adjusted in accordance with the character of the surface coating 90 on the finished paper.

From these gaging rollers 9 the web is passed 95 into the second tank 10 and through a solution which acts to convert at least a substantial portion of the silicate of soda. I have found that the second bath may be a solution of oxalic acid, formaldehyde or liquid chlorine, and aluminum sulphate; or, if preferred, instead of a liquid a gas formed of aluminum sulphate or liquid chlorine may be employed 100 as the converting agent. Where liquid is em-

ployed a second set of squeeze rollers is preferably employed.

After this converting treatment the paper is dried as by means of the second set of drying cylinders 3, and where a gloss finish is desired it is immediately passed to the calender rolls 4. As stated, the paper may be made and dried independently of the other steps. Of course, where an uncalendered product is desired, the calendering may be omitted.

The result of the treatment is a white coating and filling for the paper which may be calendered as a Satin White coated sheet produced by the usual methods. The weight of the paper is very materially increased by the treatment, the materials employed are much more economical than the china clay or Satin White commonly employed as fillers and coating, and the use of sizing and alum or other fixative commonly employed is eliminated.

A further advantage of my invention is that the coated sheet is very flexible, particularly where glycerin is employed as an ingredient, and does not dry out or become brittle.

A still further advantage is that light weight paper is rendered entirely opaque, making it practical to use light weight papers for purposes for which it has heretofore been possible to use only the heavier sheets.

The strength of the sheet is also very greatly increased.

Having thus described my invention what I claim as new and desire to secure by Letters Patent is:

1. The method of making paper comprising forming a web without sizing or precipitant, partially drying, passing the partially dried web through a liquid bath comprising silicate of soda approximately 50%, starch approximately 25%, glycerine approximately 15%, and uncolored soap approximately 10%, passing between gaging rolls, passing through a solution acting to convert a substantial portion of the silicate of soda, and drying.

2. The method of making paper comprising forming a web without sizing or precipitant, partially drying, passing the partially dried web through a liquid bath comprising silicate of soda, starch, glycerin, and soap, passing through a solution acting to convert a substantial portion of the silicate of soda, and drying.

3. The method of making paper comprising forming a web without size or precipitant, partially drying, impregnating the partially dried web with a solution comprising silicate of soda, a binder, glycerin and soap in approximately the proportions specified, subjecting to a medium acting to convert a substantial portion of the silicate of soda, drying, and calendering.

4. The method of making paper comprising forming a web without size or precipitant, partially drying, impregnating the partially dried web with a solution comprising silicate of soda, a binder, glycerin and soap in approximately the proportions specified, and subjecting to a medium acting to convert a substantial portion of the silicate of soda.

5. The method of making paper comprising forming a web without filler, partially drying, passing the partially dried web through a bath containing a substantial proportion of silicate of soda, passing through a second bath containing a chemical acting to partially convert a substantial portion of the silicate of soda, and drying.

6. A method of making paper comprising forming a web without filler, partially drying, passing the partially dried web through a bath containing a substantial proportion of silicate of soda, and subjecting to a medium acting to partially convert a substantial portion of the silicate of soda.

7. The method of treating paper consisting of passing an unsized web of paper through a liquid bath comprising silicate of soda approximately 50%, starch approximately 25%, glycerin approximately 15%, and uncolored soap approximately 10%, passing between gaging rolls, passing through a solution acting to convert a substantial portion of the silicate of soda, and drying.

8. The method of treating paper consisting of passing an unsized web of paper through a liquid bath comprising silicate of soda, a binder, and glycerin, passing between gaging rolls, passing through a solution acting to convert a substantial portion of the silicate of soda, and drying.

9. The method of treating an unsized unfilled paper comprising impregnating with a solution comprising silicate of soda, a binder, glycerin and soap, subjecting to a medium acting to convert a substantial portion of the silicate of soda, drying, and calendering.

10. The method of treating an unsized unfilled paper comprising impregnating with a solution comprising silicate of soda, a binder, and glycerin, subjecting to a medium acting to convert a substantial portion of the silicate of soda, and drying.

11. The method of treating paper consisting of impregnating an unfilled unsized paper with a solution containing a substantial proportion of silicate of soda and a binder, thereafter treating the impregnated paper to convert a substantial portion of the silicate of soda, drying, and calendering.

12. The method of treating paper consisting of impregnating an unfilled unsized paper with a solution containing a substantial proportion of silicate of soda and a binder, thereafter treating the impregnated paper to convert a substantial portion of the silicate of soda, and drying.

13. The method of treating paper consisting of impregnating paper with a solution containing a substantial proportion of silicate of soda and soap, thereafter treating the impregnated paper to convert a substantial portion of the silicate of soda, drying, and calendering.

5 14. The method of treating paper consisting of impregnating paper with a solution containing a substantial proportion of silicate of soda, thereafter treating the impregnated paper to convert a substantial portion of the silicate of soda, and drying.

10 15. In witness whereof I have hereunto set my hand.

FRANK G. CRANE.

20

25

30

35

40

45

50

55

60